

Feb. 13, 1951

R. B. HOXENG

2,541,062

UTILIZATION OF ALUMINOUS METAL ELECTRODES IN  
CATHODIC PROTECTION INSTALLATIONS

Filed Dec. 26, 1946

Fig. 1.



Fig. 2.



Fig. 3.



INVENTOR  
*Raymond B. Hoxeng*  
BY  
*George B. Todd*  
ATTORNEY

## UNITED STATES PATENT OFFICE

2,541,062

## UTILIZATION OF ALUMINOUS METAL ELECTRODES IN CATHODIC PROTECTION INSTALLATIONS

Raymond B. Hoxeng, Oakmont, Pa., assignor to  
Aluminum Company of America, Pittsburgh,  
Pa., a corporation of Pennsylvania

Application December 26, 1946, Serial No. 718,595

9 Claims. (Cl. 204—148)

1

This invention relates to installations designed to cathodically protect underground metallic structures against corrosion. The invention is specifically directed to installations of this type which utilize, as the anodic metal, aluminum or aluminum alloy having the electrical characteristics of that metal, such alloys usually being those containing upwards of 50 percent by weight of aluminum. Aluminum and such alloys are generally termed aluminous metal and such term is used herein and in the appended claims.

The essential elements and the organization of a cathodic protection system or installation are well known and will only be summarized herein to the end that the field of the invention will be clearly defined. Metallic underground structures which may require cathodic protection are of various types, including earth buried linear structures, such as pipe lines for the transport of fluids or gases, and earth buried unit structures, such as structural tower footings, tanks, oil well casings and the like. In systems designed to cathodically protect such structures against corrosion the metal of the structure is electrically connected, usually by wire or bus, to a separately buried metal piece, called an electrode, which is made of metal anodic to the metal of the underground structure. Thus is formed a galvanic cell in which the underground structure is cathode and in which the earth, in which the cell elements are buried, serves as electrolyte. In commercial installations of this character it is the object to so fashion the cell that a steady flow of current is continuously produced at high efficiency, i. e. at a low rate of consumption of the metal of the electrode which serves as anode. Where the metallic underground structure is linear or large, if of unit type, a plurality of electrodes is used separately buried at intervals along the structure and may be separately connected thereto. When an electrode is installed in such a system it is common practice to surround the buried electrode with a mixture, sometimes called a backfill, which contains chemicals which are intended to promote the action of the cell, increase its efficiency or otherwise benefit the installation.

Aluminous metal has properties recommending it for use as electrode in such a cathodic protection system. However, until recently, aluminous metal electrodes have rarely been used in such systems despite the fact that theoretical considerations indicate that aluminous metal electrodes should deliver more ampere hours per pound than most metals available for such use. In-

deed such a cathodic protection cell utilizing aluminum electrodes and operating at 75 percent efficiency is superior, on the basis of ampere hours per pound of metal, to cells utilizing electrodes made of other commercially available metals if such cells could be operated at 100 percent efficiency. This is evident upon comparison of the electrochemical equivalents of zinc, magnesium and aluminum as shown in the table on page 486 of the Transactions of the Electrochemical Society, vol. 90 (1946), in an article by H. A. Robinson on "Magnesium as a Galvanic Anode." Most buried metallic structures are constructed of metal, such as iron or steel, which is cathodic to aluminous metal, yet aluminous metal electrodes have rarely been used in such systems principally because of difficulties involved in taking advantage, under field or installation conditions, of the theoretical efficiency of aluminous metal.

An object of this invention is to provide methods and means by which the operation of aluminous metal electrodes in cathodic protection systems may be improved. A further object of the invention is to provide improved cathodic protection installations for the protection of metallic underground structures against the ravages of corrosion.

To the end of achieving these and related objects I improve the action of a cathodic protection cell embodying an aluminous metal anode by providing around the anode a mixture, or backfill, containing a mercury compound capable of yielding metallic mercury when in contact with aluminum. Usually if the backfill mixture contains at least about 0.001 percent by dry weight of the compound the results of this invention will be realized. In practice I prefer to use 0.05 to 1.0 percent by weight of a relatively insoluble mercury compound but greater amounts are not harmful and the compounds will give good results even when present in the mixture in very large amounts such as 10.0 percent. Results are not improved, however, by using excessive amounts and economic considerations usually limit the amount used to the smallest amount which will be effective under all the circumstances. One factor to be taken into consideration is the solubility of the mercury compound. It is usually preferable to use mercury compounds of limited solubility to insure that the leaching action of ground waters or moisture will not rapidly deplete the mercury compound content of the backfill mixture to a point where less than the desirable minimum is present, the occurrence of which

event may necessitate replacement of the mixture surrounding, or in contact with, the aluminous metal electrode. When relatively soluble mercury compounds are used it is, therefore, desirable to place a larger amount of compound in the mixture so that depletion by leaching below the minimum desired will not be rapid.

The backfill mixture which, in accordance with this invention is to contain the mercury compound, may otherwise be substantially chemically inactive toward the aluminous anode, i. e. it may contain as the other components earth, sand, ash, cellulosic material or other substance relatively inert to the electrode. On the other hand, the mercury compound may be added to backfill mixtures including other chemicals added to promote or improve the action of the cell of which the aluminous metal electrode is a part. For instance, good results are obtained when the mercury compound is added, in accordance with the principles of this invention, to an alkaline mixture containing inorganic halide such as that described by R. H. Brown in his copending application, Serial No. 693,593, filed August 28, 1946. In such case, however, alkalinity is not necessary to efficient results, and excellent cell operation has been achieved using a backfill mixture containing 1 to 30 percent by weight of inorganic halide and an amount of mercury salt, the balance being a carrier such as earth or other inactive material of the type above indicated.

In some cases the effectiveness of the mercury compounds, or their utility, is improved by applying the compounds directly to the surface of the aluminous metal anode using the compound in mixture with some substance which will promote adherence of the mercury compound to the anode surface. The coating thus formed, which may if desired include other substances, inert or usefully active to promote cathodic protection should contain at least 0.901 percent by coating weight of the mercury compound. The use of such coatings on the anode surface does not preclude the use of mercury compound in the backfill or other mass with which the anode is eventually surrounded.

The following examples of cathodic protection installations wherein my invention is employed are shown in the accompanying illustrations wherein.

Fig. 1 is a vertical cross sectional view through a cathodic protection cell having a bare aluminous anode surrounded by a backfill mixture containing a mercury compound of the type herein defined;

Fig. 2 is a vertical cross sectional view through a cathodic protection cell of the same type as that in Fig. 1 but having a coated aluminous anode; and

Fig. 3 is a cross sectional view of the anode on line 3-3 of Fig. 2.

Referring to Fig. 1, a hole 2 is provided in soil 1 to receive the aluminous anode 4 and the surrounding backfill 3 containing a mercury-containing compound capable of yielding mercury in contact with the buried anode. In a preferred embodiment of the invention the backfill 3 may also contain other chemicals such as alkaline materials and an inorganic halide to promote or improve the action of the cell. The anode 4 is connected by wire 5 to an underground iron pipe 6.

The cathodic protection system illustrated in Fig. 2 is similar to that in Fig. 1 in every respect except for the adherent coating 8 on anode 4

which contains the mercury compound and the backfill 7 which does not contain such a compound. If desired, the mercury compound may be included in the backfill as in the installation shown in Fig. 1. The shape of the anode 4 and the surrounding coating 8 are more clearly seen in the cross sectional view of Fig. 3.

Of the mercury compounds I prefer mercurous chloride, the preference being based on practical considerations, such as availability, cost and relative insolubility under the conditions usually obtaining in cathodic protection installations.

The advantages secured by the practice of this invention are largely those of efficiency and steady operation. Surrounded by backfills, or mixtures, containing mercury compound, the aluminous metal anode operates to steadily produce, in the galvanic cell and under installation conditions, a steady output of current at relatively high efficiencies. In practice I have observed efficiencies as high as 90 percent when mixtures embodying mercury compounds are used. In the case of one installation where various aluminous metal electrodes were installed in various types of earth for the purpose of protecting a pipe line the current output obtained was three to four times as large as obtained with conventional zinc electrodes and this output was obtained at relatively high efficiency.

Relatively efficient results in cathodic protection installations will be achieved by the use of my invention, regardless of the specific composition of the aluminous metal electrode or the specific type of mixture or backfill used to contact or surround the same. Generally, some aluminum alloys give better results as aluminous metal anodes than do others but the advantages of my invention in increasing efficiency and insuring steady cell operation will be secured, regardless of the aluminous metal anodes used, although a cell using such an anode of one specific composition will, as is known, have better overall characteristics than a cell using an aluminous metal anode of other composition. Likewise the advantages and benefits of this invention will be secured when the mixture and the aluminous metal anode are preformed into a unitary package and installed as such. An example of such a package is described in the copending application of R. B. Mears, Serial No. 705,508 filed October 25, 1946. If desired an aluminous metal anode may be coated with a mixture containing a mercury compound prior to installation, whether the electrode is used separately or as a part of a unitary package. I have found, for example, that improved aluminous metal anode operation is obtained by coating the anode with a mixture containing mercurous chloride and a protein base or a water paint or a resin emulsion paint, examples of which are known and described in standard works such as, for instance, "Protective and Decorative Coatings," volume III, published by John Wiley & Sons, Inc., New York, 1943, pages 470 and 484, prepared under the editorship of Joseph J. Mattiello. The invention is not, therefore, limited in usefulness to a specific aluminous metal electrode or to a particular form of cathodic protection system or mixture or backfill, except as indicated in the appended claims.

Having thus described my invention, I claim:

1. In a cathodic protection installation designed and operative to protect a metallic underground structure against corrosion, and comprising an underground aluminous metal electrode 75 separate from said structure, electrically con-

nected to said structure and anodic thereto, the improvement consisting in a backfill in contact with said electrode, said backfill containing at least 0.001 percent by weight of a mercury compound capable of yielding metallic mercury when in contact with said underground aluminous electrode.

2. In combination with a metallic underground structure, a separately buried aluminous metal electrode anodic to the metal of said structure and electrically connected thereto and a backfill containing at least 0.001 percent of mercury compound in contact with said electrode, said compound being capable of yielding metallic mercury when in contact with said buried aluminous electrode.

3. The method of improving the efficiency of an underground galvanic cell composed of a separately buried aluminous metal anode electrically connected to a separately buried metallic cathode which comprises maintaining in contact with said anode a material containing at least 0.001 percent by weight of mercury compound capable of yielding metallic mercury when in contact with said buried aluminous electrode.

4. An anode for use in a cathodic protection installation said anode being formed of a body of aluminous metal the surface of which bears a dry coating containing mercury compound capable of yielding metallic mercury when in contact with said aluminous body in a cathodic protection installation.

5. In a cathodic protection installation designed and operative to protect a metallic underground structure against corrosion and including an underground aluminous metal electrode separate from said structure, electrically connected to said structure and anodic thereto, the improvement consisting in an alkaline backfill in contact with said electrode, said backfill containing at least 0.001 percent by weight of mercury compound capable of yielding metallic mercury when in contact with said underground aluminous electrode.

6. A unitary package for use in cathodic protection of underground metallic structures comprising an aluminous metal electrode in contact with a dry mixture containing at least 0.001 percent by weight of mercury compound capable of yielding metallic mercury when in contact with said aluminous electrode in a cathodic protection installation.

7. In a cathodic protection installation designed and operative to protect a metallic underground structure against corrosion and comprising an underground aluminous metal electrode separate from said structure, electrically connected to said structure and anodic thereto, the improvement consisting in the fact that the surface of said electrode is covered, at least in part, with a mercury compound capable of yielding metallic mercury when in contact with said underground aluminous electrode.

8. In combination with a metallic underground structure, a separately buried aluminous metal electrode anodic to the metal of said structure and bearing on its surface a mercury compound capable of yielding metallic mercury when in contact with said buried aluminous electrode.

9. In combination with a metallic underground structure, a separately buried aluminous metal electrode anodic to the said structure and electrically connected thereto and a backfill containing at least 0.001 per cent of mercury compound in contact with said electrode, said compound being capable of yielding metallic mercury when in contact with said buried aluminous electrode, and the ampere output per hour of said electrode being greater than the ampere output per hour of the same electrode in the described combination with said structure but not in contact with a backfill containing said mercury compound.

RAYMOND B. HOXENG.

#### REFERENCES CITED

The following references are of record in the file of this patent:

#### FOREIGN PATENTS

| Number  | Country       | Date          |
|---------|---------------|---------------|
| 437,536 | Great Britain | Oct. 31, 1935 |

#### OTHER REFERENCES

- “Treatise on Inorganic and Theoretical Chemistry,” by J. W. Mellor, vol. 5 (1924), page 221.
- “Transactions of the American Electrochemical Society,” vol. 52 (1927), page 360.
- “Proceedings of the first annual meeting of the National Association of Corrosion Engineers,” (1944), pages 61 through 66.
- “Status of Cathodic Protection Lines in 1941,” by Logan, pages 6 and 7.